

C. T. FULLER,  
METAL DRAWING DIE,  
APPLICATION FILED NOV. 4, 1916.

1,297,825.

Patented Mar. 18, 1919.

Fig.1.



Fig.2.



Inventor:  
Carl T. Fuller,  
by *Alon G. Durso*  
His Attorney.

# UNITED STATES PATENT OFFICE.

CARL T. FULLER, OF NUTLEY, NEW JERSEY, ASSIGNOR TO GENERAL ELECTRIC COMPANY, A CORPORATION OF NEW YORK.

## METAL-DRAWING DIE.

1,297,825.

Specification of Letters Patent. Patented Mar. 18, 1919.

Application filed November 4, 1916. Serial No. 129,478.

*To all whom it may concern:*

Be it known that I, CARL T. FULLER, a citizen of the United States, residing at Nutley, county of Essex, State of New Jersey, have invented certain new and useful Improvements in Metal-Drawing Dies, of which the following is a specification.

In drawing tungsten which has been rendered ductile by suitable manipulation and mechanical working in a manner now well known in the art, drawing dies of selected diamonds have hitherto been used, as a diamond of good quality was the only material known which was hard enough to resist for any length of time the abrading action of the hard tungsten and was also strong enough to withstand the stresses which tend to split the die. These dies are very expensive, particularly for large wire, and wear away quite rapidly, so that after a moderate length of wire has been drawn, the opening through the die is too large. Many dies are also lost by splitting or breaking during the drawing operation.

The object of my invention is to reduce the expense of dies in drawing tungsten and similar hard refractory metal. Another object is to provide a cheap and easily manufactured drawing die which will be suitable for drawing tungsten wire, particularly those sizes which are drawn hot.

I tested metal drawing dies made of the best grades of tungsten tool steel and also of pure tungsten sintered and consolidated as much as possible and found that none of these dies would last long enough to make it worth while to use them. All of them were enlarged so rapidly by the abrasion and wearing away of the walls of the opening that each length of wire drawn was appreciably larger than the preceding length, and in some cases the diameter of a comparatively short length of wire was appreciably greater at the end than at the beginning. My tests demonstrated that neither the best tungsten steel available nor pure tungsten was of any value for making drawing dies for tungsten wire.

In accordance with my invention I consolidate finely divided tungsten by means of

5% to 15% of iron into a dense homogeneous drawing die, which has such tensile strength that it does not split or break when tungsten is drawn through it, and which has the remarkable and unexpected property 55 of resisting abrasion so well that the opening through it remains of substantially the same size during the drawing of great lengths of tungsten wire, although both the wire and the die are at red heat. A drawing die constructed in accordance with my invention can be made for a small fraction of the cost of a diamond die of the same size and its life is usually a large fraction of that of the diamond die, so that a large saving 60 in the cost of drawing tungsten wire is effected by using these drawing dies, particularly for hot drawing the wire to reduce it from the size at which it leaves the swaging machines to the smaller sizes of wire 70 which may be drawn below red heat in diamond dies without excessive expense for dies.

Merely for purposes of illustration I have shown in the accompanying drawing one 75 form in which my invention may be embodied and in which Figure 1 is a plan view of one form of die, and Fig. 2 is a longitudinal section through the die and its holder. This particular drawing die 1 is in 80 the form of a thick disk or short cylinder having a central opening 2. I prefer to mount this die loosely in a suitable holder such as a strong steel block 3 having a pocket 4 deep enough to hold the die securely and 85 slightly larger than the greatest diameter of the die. The bottom of the pocket has a central opening 5 considerably larger than the opening 2 of the die. I prefer to so shape the die and the holder that the die is 90 supported near its center. For example, if the die is flat, the bottom of the pocket 4 may be slightly convex, as shown at 6, or if the pocket has a flat bottom the surface of the die may be slightly convex. In either 95 case the pull of the wire passing through the die in the direction of the arrow seats the central portion of the die firmly on the bottom of the pocket. The die may be held in the pocket 4 by a retaining ring 7. 100

In operation the holder and die are heated to about 600° C., and the tungsten wire is also heated so that it is red hot when entering the die and is still red hot when emerging from it. Lower temperatures may be used as the wire becomes smaller, but the best results are obtained with these dies when the wire is drawn hot.

To make the drawing die, I mix finely divided tungsten with finely divided iron to produce a homogeneous powder containing from 5% to 15% of iron, and press this powder in a strong steel mold by a hydraulic press into a disk of the approximate size of the finished die. The pressed disk of powder is sufficiently coherent to retain its shape if it is handled with care. The disk of pressed powder is then placed in a boat or on a strip of suitable material, such as molybdenum, and introduced into an electric furnace comprising a refractory tube of porcelain or alundum with a heating coil wound on it. The disk is heated or fired in the furnace at as high a temperature as possible, usually about 1800° C. in an atmosphere of hydrogen for about one-half hour. At this temperature and under these conditions the pressed disk does not melt down or lose its shape, but the particles of tungsten are completely consolidated by the iron into a dense coherent block of metal, too hard to be machined, and having even at red heat such tensile strength and remarkable resistance to abrasion that the die made from it can safely be set loosely in the holder 3, as shown in Fig. 2, and used at red heat without danger of splitting.

To facilitate making the die a perforation smaller than the opening in the finished die may be made through the disk of pressed powder and then be enlarged to the proper size after the disk has been fired.

I have found that the best results are obtained with a mixture composed of about 45 90% by weight of powdered tungsten and 10% by weight of powdered iron, although good results are obtained where the iron is as little as 5% or as great as 15%. If these limits are exceeded the die does not have the 50 long life and resistance to abrasion characteristic of the die having the proper amount of iron.

While I do not wish to advance any theory as to the nature of the metal forming the die, it is highly probable that the iron and the tungsten form a solid solution which is homogeneous at the temperature attained in the electric furnace and also at all lower temperatures, particularly at about red heat.

60 I have secured the best results by making the dies from unwrought tungsten metal obtained in the form of powder by reducing tungstic oxid, arranged in a layer not more

than an inch deep, in a refractory tube through which a current of pure, dry hydrogen is passed while the temperature of the tube is slowly raised so that in six or seven hours it attains a temperature of 65 900° or 1100° C. The object of this procedure is to secure the tungsten metal in the form of 70 a grayish powder, such as is used in manufacturing drawn wire filaments, and coarser than the very black impalpable tungsten powder such as was generally used in manufacturing lamp filaments by the squirting 75 process. This tungsten metal may to advantage be the same as is commonly used to make ductile tungsten. This metal contains about 1% or less of thorium oxid.

The iron and the trungsten may be intimately mixed in various ways, but the procedure which I prefer and by which I have obtained the best results, is as follows: 500 grams of ferrous sulfate is dissolved in about four liters of water and ammonia water is 80 added gradually to the solution while the whole mass is agitated by means of an air jet until the ferrous hydrate is precipitated. About 1 liter more of water is added and the precipitate allowed to settle, after which the 85 precipitate is washed, preferably by agitating it with water, permitting it to settle, and siphoning off or decanting the supernatant liquid. The ferrous hydrate is washed until free from ammonium salts. The moist ferrous hydrate is then poured into a porcelain evaporating dish containing 900 grams of the powdered tungsten metal prepared as above described. The contents of the dish are well mixed and then dried, preferably on 95 a hot plate or by steam. The resultant dried mass is then placed in shallow sheet iron boats in charges of about 300 grams each, and reduced in hydrogen gas in an electric furnace comprising a refractory tube 100 through which the hydrogen flows. This tube is kept, at its hottest part, at a temperature from 23 to 25% of the temperature of the filament of a carbon lamp operating at an efficiency of 3.1 watts per candle. The 105 hydrogen should be well dried by sulfuric acid and phosphorus pentoxid. The furnace should be so arranged that the sheet iron boats pass through the hot zone of the furnace at the rate of about one-half inch per minute and on into a cool end portion, which may be of iron and water cooled.

110 After the boats are removed from the cool end of the furnace, the contents should be placed quickly in glass stoppered bottles, care being exercised to prevent the reduced die metal from burning in the air as it is quite pyrophoric. In the course of a few hours the dry metal may with safety be sieved and bolted to produce a mass of fine 115 powder containing approximately 10% iron

and 90% tungsten and very suitable for the manufacture of metal drawing dies by pressing and firing in the manner above described.

- 5 5. What I claim as new and desire to secure by Letters Patent of the United States, is,—  
1. A metal die for wire drawing at about red heat consisting of an alloy of iron and

tungsten containing between 5% and 15% of iron.

2. A metal die for wire drawing consisting of an alloy of iron and tungsten containing substantially ten per cent. of iron.

In witness whereof, I hereunto set my hand this second day of November, 1916.

CARL T. FULLER.